

# United States Patent [19]

Abiko et al.

[11] 3,929,618

[45] Dec. 30, 1975

[54] **PROCESS FOR THE CONVERSION OF HYDROCARBON FRACTIONS CONTAINING CONDENSED-RING POLYCYCLIC AROMATIC HYDROCARBON**

[75] Inventors: **Shiro Abiko; Kazuo Yorihiro**, both of Yokkaichi; **Toshiyuki Sugihara; Masakazu Hanawa**, both of Ami, all of Japan

[73] Assignee: **Mitsubishi Co., Petrochemical Ltd., Japan**

[22] Filed: **Mar. 12, 1974**

[21] Appl. No.: **450,395**

|           |         |                    |         |
|-----------|---------|--------------------|---------|
| 3,364,150 | 1/1968  | Hughes .....       | 252/439 |
| 3,437,586 | 4/1969  | Weisz .....        | 208/110 |
| 3,640,819 | 2/1972  | Watkins .....      | 208/111 |
| 3,644,200 | 2/1972  | Young .....        | 208/120 |
| 3,694,345 | 9/1972  | Bittner .....      | 208/111 |
| 3,778,365 | 12/1973 | Hamner et al. .... | 208/111 |
| 3,824,180 | 7/1974  | Hilfman .....      | 208/111 |

*Primary Examiner*—Delbert E. Gantz

*Assistant Examiner*—G. E. Schmitkons

*Attorney, Agent, or Firm*—Robert E. Burns; Emmanuel J. Lobato; Bruce L. Adams

## [30] Foreign Application Priority Data

Mar. 15, 1973 Japan..... 48-30205

[52] U.S. Cl..... 208/111; 208/73; 252/455 Z; 252/456; 252/464

[51] Int. Cl. 2..C10G 13/06; C10G 37/02; B01J 29/12

[58] Field of Search ..... 208/111, 72, 73, 58, 61; 252/455 Z, 456

## [57]

## ABSTRACT

Process for the catalytic hydrogenative ring opening of hydrocarbon fractions containing condensed ring polycyclic hydrocarbons in the presence of a new catalyst comprising a carrier of NaY-type zeolite, at least 60% (mol) of the sodium ions contained in said zeolite having been exchanged with nickel ion, supported thereon nickel, tungsten and vanadium. The new catalyst exhibits an excellent hydrogenative ring opening activity.

## [56] References Cited

### UNITED STATES PATENTS

3,132,087 5/1964 Kelley et al..... 208/60

9 Claims, No Drawings

**PROCESS FOR THE CONVERSION OF  
HYDROCARBON FRACTIONS CONTAINING  
CONDENSED-RING POLYCYCLIC AROMATIC  
HYDROCARBON**

**BACKGROUND OF THE INVENTION**

**1. Field of The Art**

The present invention relates to a process for the hydrogenative ring opening of polycyclic hydrocarbons. In particular, it is concerned with a process for the hydrogenative ring opening of polycyclic hydrocarbons or heavy hydrocarbon oils containing a large amount of polycyclic hydrocarbons which comprises contacting these hydrocarbon materials with a novel catalyst having a high activity under highly pressurized hydrogen.

Such type of catalyst have, heretofore, been used in hydrocracking by which gasoline with a high octane rating is to be produced. The hydrocracking process comprises subjecting heavy oils, particularly gas oil fractions to cracking under pressurized hydrogen, and the principal reactions involved therein are chain cleavage and isomerization of paraffins and hydrogenation and subsequent ring opening of aromatics contained therein. (See, for example, A. Voohries et al: Advances in Petroleum Chemistry and Refining Vol. VIII pp. 169. Interscience Publishers, New York 1964.) Such reactions may be useful as a pre-treatment means in, for example, thermal-cracking of heavy oils by which raw materials for chemicals are to be produced. For instance, it is known that when the heavy oils are thermally cracked, the aromatic hydrocarbons contained therein undergo no ring opening under a cracking temperature lower than 900°C and, is even dehydrocondensed to form biphenyl type compounds which are retained in the heavy residue oils, so that fuel oils are largely produced and useful light olefins or monocyclic aromatics are not obtained. It is also known that partially hydrogenated condensed ring aromatic hydrocarbons are, for the most part, converted to original aromatic hydrocarbons (in this case naphthalene) through a dehydrogenation reaction when they are subjected to heat treatment, (for example, with tetratin, see L. Alexander et al: J. Chem. Soc, B9 1733-9 (70). This fact indicates that hydrogenative ring opening is essential for the pre-treatment of heavy oil for thermal cracking or conversion of heavy oils into light oil.

**2. Prior Art**

In the conventional studies to produce light fractions of hydrocarbons using catalyst for hydrocracking, most of the hydrocarbons used are paraffin hydrocarbons. The conversion of aromatic hydrocarbons are only disclosed in V. C. Rumohr et al: Erdoel und Kohle Erdgas - Petrochemie 25 309 (1972) and paring reaction is disclosed in Sullivan: J. Am. Chem. Soc. 83, 1156 (1956). The former is directed to the production of a large amount of naphthalene fractions from anthracene, phenanthrene, and the latter is concerned with the cleavage of the side chains of polyalkylbenzene. Studies concerning the hydrogenative ring opening of polycyclic aromatics have been little known.

Although some patents disclose catalysts for the conversion of hydrocarbons which contain the same components as those of the catalyst of the present invention as hereinafter detailed, these catalysts have been used for the production of high octane gasoline and they are

not shown to be useful particularly for the hydrogenative ring opening of polycyclic aromatic hydrocarbons. As is apparent from the comparative example in experiments as hereinafter described, the catalysts for hydrocracking commercially available do not necessarily produce excellent results in the tests for such ring opening performance. On the other hand, several patents teach catalyst compositions for hydrocracking containing vanadium as a component, but there are disclosed only a few catalysts having excellent cracking activity wherein zeolite is used as a solid acid carrier. None of these patents gave detailed description of the catalyst containing the zeolite carrier (for example, see U.S. Pat. Nos. 2,817,626; 2,839,450; 3,383,306; 3,437,586 and 3,640,819 and Japanese Pat. Publication No. 35613/71).

**SUMMARY OF THE INVENTION**

The present invention relates to a process for the production of monocyclic aromatics and alkyl naphthenes with a high yield from hydrocarbons containing a large amount of fused-ring aromatics and the desulfurization of said hydrocarbon fractions in the production of monocyclic aromatic and alkyl naphthenes by effecting the hydrogenative ring opening under pressurized hydrogen in the presence of a catalyst with hydrocracking metals Ni, W and V supported on a carrier of zeolite Y with nickel ion exchanged therewith.

Accordingly, the process for the conversion of hydrocarbon fractions containing polycyclic aromatic hydrocarbon is characterized in that the catalyst hydrogenative ring opening of hydrocarbon fractions containing at least 10% (by weight) polycyclic aromatic hydrocarbons is carried out in the presence of a catalyst comprising a carrier of Y-type zeolite, at least 60% (mol) of the sodium ions contained in said zeolite having been exchanged with nickel ion, supported thereon 1 to 25% nickel, 1 to 20% tungsten and 0.1 to 5% vanadium based on the weight of the carrier + these metals.

In view of the above, the distinctive characteristics of the present invention are that the zeolite Y which has undergone exchange with nickel ion is used as a carrier and vanadium (and nickel and tungsten) is contained as a catalyst metal component, and for such characteristic, the catalyst of the present invention results in a great improvement in hydrogenative ring opening activity (see the comparative Examples as hereinafter described).

**DETAILED EXPLANATION OF THE INVENTION**

**1. Catalyst**

**1. Kind of Catalyst**

One feature of the catalyst according to the present invention is that the carrier is Na Y-type zeolite which have undergone exchange with nickel ion.

The zeolite Y used in the present invention is a synthetic zeolite having the structure of sodalite which may be commercially available. The zeolite has an atomic ratio of Si/Al of 2.2 to 3.0 and belongs to the Group 4 of the classification by D. W. Breck et. al. (See, D. W. Breck: Molecular Sieve Zeolites, Advances in chemistry Series 101, Am. chem. Soc. Washington D.C. (1971)).

The catalyst used in the present invention is required to have nickel which substitutes for sodium ions in a zeolite carrier and also nickel supported on the carrier.

The catalyst according to the present invention may be used in a sulfided form, and it is usually sulfided in practice.

## 2. Preparation of Catalyst

### Preparing of Carrier

i. A predetermined amount of dry zeolite Y is subjected to ion exchange treatment in a solution of NH<sub>4</sub>Cl. The NH<sub>4</sub>Cl solution used is such that NH<sub>4</sub><sup>+</sup> ions are present in an amount of 0.5 to 3 times that of sodium ions contained in the zeolite. The zeolite Y in the form of powder or pellet is immersed in the afore-mentioned solution and heated to a temperature of 80 to 90°C and left with stirring for 1 to 6 hours. At the end of that time, the resulting mixture is filtered and thoroughly washed with pure water or the solvent.

The ion exchange operation as stated above is repeated 3 to 6 times using a fresh NH<sub>4</sub>Cl solution at every operation, whereby 90 to 95% of the Na ions contained in the zeolite is replaced by NH<sub>4</sub><sup>+</sup> ions. The zeolite Y thus exchanged is called NH<sub>4</sub>-Y.

ii. A predetermined amount of dry zeolite Y is subjected to ion-exchange treatment in an aqueous solution of salts of nickel. Any kind of salts of nickel which are water-soluble may be used. Nickel nitrate, nickel chloride and the like are usually used. The content of the Ni ions contained in the aqueous solution of nickel salts is usually in the range of from 0.5 to 3.0 times that of Na ions. With less amounts of Ni ions, the degree of ion exchange is decreased, so that the number of exchanging operations should be increased. The ion exchange is carried out according to the same procedure described in (i). The repeated ion exchange over 3 to 6 times could replace 75 to 80% of the sodium ions contained in the zeolite with Ni ions. As is seen in Examples as hereinafter described, at least 60% of the sodium ions should be replaced with Ni ions. The zeolite Y thus replaced with Ni ions is called Ni-Y.

iii. The NH<sub>4</sub>-Y ion exchanged according to the procedure described in i. is ion exchanged with Ni ions using the same ion exchange method as that described in (ii). The resultant zeolite is called Ni-NH<sub>4</sub>-Y.

### Support Of Metal Component And Sulfiding

The afore-mentioned NH<sub>4</sub>-Y, Ni-Y or Ni-NH<sub>4</sub>-Y as a used carrier is impregnated with the compounds which are sources of metal components in the form of, preferably, a solution (particularly, an aqueous solution), respectively. Nickel, tungsten and vanadium are deposited on the carrier in the weight ratio of 1 to 25:1 to 20:0.1 to 5, and, preferably, 6 to 20:1 to 10:1 to 2, respectively, calculated on the basis of the assumption that the total of the carrier and the metals amounts to 100.

As a source of nickel, any compounds, preferably, water soluble compounds such as nickel nitrate, which forms metallic nickel on thermal decomposition, may be used. The nickel nitrate may be used in the form of 60 a slurry.

As a source of tungsten, any compounds, preferably, water-soluble compounds such as ammonium silicotungstate or paratungstate, which form metallic tungsten or tungsten oxides upon thermal decomposition, 65 may be used. As a source of vanadium, any compounds, preferably water-soluble compounds such as ammonium metovanadate, which form metallic vana-

dium or vanadium oxides upon thermal decomposition, may be used.

These compounds may be used as the sources of the metal components of the catalyst in any type of combination without having appreciable effect on the catalytic performance.

The supporting of the metal components on the carrier is carried out by mixing an aqueous solution or slurry of the respective salts of Ni, W and V with the ion exchanged zeolite Y as stated above and evaporating the resulting mixture to dryness. The mixing may be carried out by treating the mixture in a kneader for 0.5 to 5 hours.

The mixture is then dried in a dryer at a temperature in the order of 90° to 150°C. Thereafter, the dried mixture is calcined in an atmosphere of air or an inert gas such as nitrogen, helium, argon and the like in a muffle furnace. In this case, in order to prevent the occurrence of local high temperatures due to the decomposition of the salts, the content is gradually heated from room temperature to a temperature of 200° to 400°C and kept at that temperature for 0.5 to 3 hours, after which it is heated at a temperature of 480° to 550°C for a further 3 hours.

Following this, the mixture is reduced in a stream of hydrogen at a temperature of about 350° to 450°C for about 0.1 to 5 hours and then pre-sulfided in a stream of hydrogen containing 1 to 15% (by volume) H<sub>2</sub>S, CS<sub>2</sub>, thiophene and the like. This sulfiding is carried out in a stream of hydrogen containing H<sub>2</sub>S, CS<sub>2</sub>, thiophene and the like at a temperature of about 200° to 400°C for about 1 to 60 minutes. After the sulfiding, the catalyst is cooled to room temperature in an atmosphere of nitrogen. Further, the sulfiding of the catalyst may also be effected by adding a simple organosulfur compound such as thiophene or carbon disulfide at the starting of operation in the hydrocarbon conversion process.

The catalyst thus obtained may be shaped into a tablet and other shaped products, if desired. The shaping may be carried out before the impregnation of the compounds of the catalytic metal component sources, but it is, preferably, carried out after the impregnation, and more preferably after the calcining. The shaping may be carried out using a suitable binder such as silica-alumina, if desired.

## 2. Conversion of Hydrocarbon

### 1. Reaction Conditions:

50 The reaction conditions of the hydrogenative ring opening of condensed ring aromatic are as follows:

#### i. Reaction temperature

The temperature at which the reaction is carried out may preferably be any temperature within the range of 250° to 500°C, and more preferably 350° to 470°C. With higher temperatures gasification is increased, while with lower temperatures conversion is decreased. The optimum temperature may be determined depending upon the feed of charge stocks used.

#### ii. Reaction pressure:

The pressure of hydrogen at which the reaction is conducted may be any pressure in the range of 10 to 200 kg/cm<sup>2</sup>, and preferably, 50 to 150 kg/cm<sup>2</sup>. The higher the pressure the higher the conversion, but at pressures above 100 kg/cm<sup>2</sup> the increase in the conversion slopes down. Therefore, the use of a pressure of from 60 to 120 kg/cm<sup>2</sup> is more preferably in usual operations.

## iii. Flow rate of hydrogen:

The higher the flow rate of hydrogen the greater the conversion, but the flow rate usually used in the range of 500 to 5,000 [Hydrogen gas volume/feed liquid volume] with respect to the flow rate of the charge stock. The preferred flow rate ranges from 800 to 1,500 [gas volume/liquid volume].

## iv. LHSV (liquid hourly space velocity)

The LHSV employed in the process is usually in the range of 0.5 to 6/hr, and preferably 1 to 4/hr.

## 2. Hydrocarbon Charge Stock

The hydrocarbon charge stock used in the present invention is hydrocarbon fractions containing not less than 10% (by weight) and preferably 20% (by weight) of condensed ring aromatic hydrocarbons.

The term "condensed ring aromatic hydrocarbons" as herein used signifies hydrocarbons which contain at least one benzene ring in the structure of the condensed ring and have, preferably, not less than 10 carbon atoms. Illustrative examples of such condensed ring aromatic hydrocarbon include naphthalene, methylnaphthalenes, anthracene, phenanthrene, pyrene, acenaphthene, tetralin and the like and alkylderivatives thereof.

The hydrocarbon fractions containing not less than 10% of condensed ring aromatic hydrocarbons include FCC recycle oil, vacuum gas oil, straight run heavy gas oil, residue of thermal cracking, coal tar gas oil and the like.

The content of the condensed ring aromatic hydrocarbons present in these hydrocarbon fractions is represented by the weight ratio of aromatic ring forming carbon which is determined from the intensity ratio of aromatic ring constituting hydrogen to other hydrogen by means of a nuclear magnetic resonance (NMR) method.

## 3. Reaction Result

The hydrogenative ring opening of heavy oils containing a large amount of condensed ring aromatics through the use of the aforementioned catalysts enables obtaining of monocyclic aromatics and naphthenes with a high yield.

More specifically, when  $\alpha$ -methylnaphthalene as a model of the condensed ring aromatics is, for example, subjected to hydrogenative ring opening to give monocyclic aromatics and naphthenes, the yield of the monocyclic products is 20% (by weight) with the commercially available catalysts Ni—W/SiO<sub>2</sub>.Al<sub>2</sub>O<sub>3</sub> suitable for hydrocracking while with the Ni—W—V/NiY catalyst of the present invention the monocyclic products can be obtained with a yield of 80% (by weight). The reaction conditions under which the comparative experiments were conducted included a temperature of 450°C, a pressure of 80 kg/cm<sup>2</sup> and a LHSV of 2 hr<sup>-1</sup>, and the comparative data were mainly taken 2 hours after the  $\alpha$ -methylnaphthalene was passed over the catalysts.

## 4. Experimental Examples

## EXAMPLE-1

## (Catalyst preparation)

## Catalyst preparation procedure (1)

In this procedure, the catalyst is prepared by using an indirect nickel exchange method which will be given hereunder.

500 g of dry zeolite Y was immersed in 2l of an aqueous solution of 107 g NH<sub>4</sub>Cl in water and then, the zeolite was ion exchange treated with stirring while maintaining the mixture at a temperature of 80° to 90°C. After 3 hours, the resulting mixture was filtered and the resulting exchanged zeolite was washed with water, after which the washed zeolite was again subjected to ion exchange treatment in a fresh NH<sub>4</sub>Cl aqueous solution of the same concentration in the same manner described above. When such ion exchange treatment was repeated 3 times, 73% of Na<sup>+</sup> ions was replaced by NH<sub>4</sub><sup>+</sup> ions. The product thus obtained is called NH<sub>4</sub>—Y (1).

The NH<sub>4</sub>—Y(1) was baked in a muffle furnace at 500°C for 1 hour, and then shaped into a pellet having a size of 5 mmΦ by means of a pelletizing machine.

After shaping, to 30g of NH<sub>4</sub>—Y(1) was added 200cc of an aqueous solution of 37.4 g of nickel nitrate (6 hydrate) and 1.06g of ammonium paratungstate.

30 The resulting mixture was evaporated to dryness to impregnate the NH<sub>4</sub>—Y (1) with the solution, and the impregnated NH<sub>4</sub>—Y (1) was dried in a dryer at a temperature of 110°C for 24 hours. After drying, the dried product was calcined at 550°C for 3 hours. The

35 catalyst so produced is called Ni—W/NH<sub>4</sub>—Y(1). On the other hand, 30 g of NH<sub>4</sub>—Y(1) after being shaped was impregnated with an aqueous solution containing 37.4 g of nickel nitrate (6 hydrate), 1.06g of ammonium paratungstate and 0.386 g of ammonium vanadate and calcined according to the same manner as that described above. The catalyst so produced is called

40 Ni—W—V/NH<sub>4</sub>Y(2).

## Catalyst preparation procedure (2)

45 In this procedure, the catalyst is prepared by using a direct nickel exchange method which will be given hereunder.

500 g of dry zeolite is added to a nickel salt aqueous solution of 300 g Ni (NO<sub>3</sub>)<sub>2</sub>.6H<sub>2</sub>O in 2l of pure water to form a slurry. The slurry was ion exchange treated with stirring while maintaining it at a temperature of 80° to 90°C. After 3 hours, the resulting product was filtered and the resulting exchanged zeolite was washed with water and dried. The dried zeolite was again mixed with

55 a fresh Ni(NO<sub>3</sub>)<sub>2</sub> aqueous solution having the same concentration as that of the first solution, and the resulting mixture was left, water washed and filtered and the resulting exchanged zeolite was dried in the same manner as that described above.

60 Such ion exchange treatment was repeated three times. The drying was carried out in a drier at 110°C for 24 hours. The ion-exchange treatment resulted in the replacement of 75 to 77.5% Na ions with Ni ions. The Ni-exchanged zeolite Y so produced is called Ni—Y(3).

To 15 g of Ni—Y(3) was added 100 ml of an aqueous solution containing 6.64 g of nickel nitrate hexahydrate, 0.5297g of silicotungstic acid and 0.1926 g of

ammonium metavandate and the resulting mixture was evaporated to dryness to attain the impregnation of Ni, W, and V components. After the impregnated Ni-Y(3) was dried at a temperature of 110°C for 24 hours, the dried Ni-Y(3) was introduced into a muffle furnace and first calcined at a temperature of 300°C for 1 hour, after which the temperature was gradually raised to 500°C and calcining was further carried out at that temperature for 3 hours. After the grinding of the calcined grains, the ground product was shaped into pellets having a size of 5 mmφ by means of a pelletizing machine. The pellets were baked at a temperature of 500°C for 1 hour. The catalyst so obtained is called Ni-W-V/Ni-Y(3).

Chemical analysis showed that the Ni-W-V/Ni-Y(3) catalyst contained 2.2 weight percent sodium, 15

As can be seen from Table 1, the comparison of the catalyst Ni-W/NH<sub>4</sub>Y(1) with the catalyst Ni-W-V/NH<sub>4</sub>Y(2), both catalysts being prepared according to the catalyst preparation procedure (1), indicates that the addition of vanadium results in a substantial improvement in hydrogenative ring opening activity.

### EXAMPLE-3

#### (Hydrocarbon conversion)

Using the catalyst prepared according to the catalyst preparation procedure 2, described in Example-1, hydrogenative ring opening reaction was carried out under the same conditions as described in Example 2.

The results obtained 10 hours after the charge stock was passed over the catalyst are shown in Table 2.

Table 2

|                     | Catalyst       | Percent conversion of α-methylnaphthalene | Percent yield of monocyclic aromatics and decalin |
|---------------------|----------------|-------------------------------------------|---------------------------------------------------|
| Present Invention   | Ni-W-V/Ni-Y(3) | 85                                        | 78                                                |
| Comparative Example | Ni-W/Ni-Y      | 83                                        | 70.5                                              |
|                     | Ni-V/Ni-Y      | 80                                        | 65                                                |

16.2 weight percent nickel (including Ni in the carrier Ni-Y), 1.6 weight percent tungsten and 1.6 weight percent vanadium, calculated on the basis of the catalyst dried at 200°C for 2 hours. (since approximately 77 molar % of sodium ion was exchanged with nickel ion in the carrier NiY(3), the amount of impregnated nickel is 10.5% by weight.)

### EXAMPLE-2

#### (Hydrocarbon conversion)

Hydrogenative ring opening reaction was performed using α-methylnaphthalene (which was selected as a model of the condensed ring aromatics) as a hydrocarbon oil charge. Prior to the reaction, all the catalysts were reduced in a stream of hydrogen at a temperature of 400°C for 3 hours, and then cooled in a stream of nitrogen to 300°C and sulfided in a stream of a mixture of 10% (by volume) of H<sub>2</sub>S and 90% (by volume) of hydrogen:

The efficiency of the catalysts was compared at undegiven reaction conditions a temperature of 450°C, a pressure of 80 kg/cm<sup>2</sup>, a LHSV of 2 hr<sup>-1</sup>, a catalyst amount of 15cc and H<sub>2</sub>/oil = 1,000 Nm<sup>3</sup>/Kl. The comparative data were obtained 10 hours after the α-50 methylnaphthalene was passed over the catalysts.

The results are shown in Table 1. In this connection, the yields of monocyclic aromatics and decalin are represented by weight percent based on the weight of the charge stock.

30 As is apparent from Table 2, the absence of W or V affects conversion very little, but causes reduction in ring opening activity. The other conversion products include predominantly indane, tetralin and methyl derivatives thereof which are undesirable for the purpose of the present invention.

### EXAMPLE-4 (Hydrocarbon conversion)

35 Using the catalysts of Example 1 wherein the degree of ionexchange of the Ni-Y carrier was varied as indicated in Table 3, hydrogenative ring opening reaction was performed according to the same procedure described in Example 2 and the comparison of catalysts performance was carried out 2 hours after the charge stock was passed over the catalysts.

40 The results are shown in Table 3. The higher the ionexchange the better the hydrogenative ring opening activity, and it is clear that the degree of ionexchange of not less than 60% is required.

Table 3

| Ni ion exchange %        | Yield of ring opened product (including decalin) %          |
|--------------------------|-------------------------------------------------------------|
| 40                       | 47                                                          |
| 60                       | 71                                                          |
| 69                       | 75                                                          |
| 77                       | 82                                                          |
| Experimental conditions: | Catalyst Temperature Ni-W-V/Ni-Y 425°C 80kg/cm <sup>2</sup> |

Table 1

|                     | Catalyst                                                 | Percent conversion of α-methylnaphthalene | Percent yield of monocyclic aromatics and decalin |
|---------------------|----------------------------------------------------------|-------------------------------------------|---------------------------------------------------|
| Comparative Example | Ni-W/NH <sub>4</sub> Y(1)                                | 66                                        | 47                                                |
| Present Invention   | Ni-W-V/NH <sub>4</sub> Y(2)                              | 82                                        | 70                                                |
| Comparative Example | Ni-W/SiO <sub>2</sub> , Al <sub>2</sub> O <sub>3</sub>   | 52                                        | 17                                                |
|                     | Ni-W-V/SiO <sub>2</sub> , Al <sub>2</sub> O <sub>3</sub> | 65                                        | 23                                                |

## EXAMPLE 5

In this example, hydrogenative ring opening reaction was carried out using various catalysts prepared according to different preparation procedures.

The reaction conditions were identical to those described in Example 2, and the data were obtained 10 hours after the charge stock was passed over the catalysts.

Table 4

| Style of catalyst preparation procedure | Percent conversion of $\alpha$ -methylnaphthalene | Percent yield of monocyclic aromatics and decalin |
|-----------------------------------------|---------------------------------------------------|---------------------------------------------------|
| 1 Exchange, 2 Impregnation, 3 Shaping*  | 82                                                | 72                                                |
| 1 Shaping, 2 Exchange, 3 Impregnation** | 76                                                | 65                                                |
| 1 Exchange, 2 Shaping, 3 Impregnation** | 85                                                | 67                                                |

\*Ni-N-V/Ni-Y prepared by the catalyst preparation procedure (2)

\*\*Ni-W-V/Ni-Y prepared by altering the order of shaping.

As is clear from Table 4, the procedure according to catalyst preparation procedure (2) described above, namely, the procedure of "1 Exchange, 2 Impregnation, 3 Shaping" is most preferable.

## COMPARATIVE EXAMPLE - 1

In this example, hydrogenative ring opening reaction was carried out using Ni-W-V/M-Y catalysts in which M-Y was varied as indicated in Table 5. Ni-Y was found to be the most useful carrier.

The catalyst preparation procedure and the hydrocarbon conversion process were similar to the catalyst preparation procedure (2) and Example 2, respectively. The conditions of the hydrocarbon conversion process were as follows: Temperature: 450°C, pressure: 80 kg/cm<sup>2</sup>, LHSV: 2 hr<sup>-1</sup>. The data were obtained 1.5 hours after the charge stock was passed over the catalysts. The results are shown in Table 5.

Table 5

| Metal ion used for exchange | Exchange (%) | Yield of ring opened product (including decalin) |
|-----------------------------|--------------|--------------------------------------------------|
| Ni <sup>2+</sup>            | 75           | 83                                               |
| Ca <sup>2+</sup>            | 87           | 44                                               |
| Al <sup>3+</sup>            | —            | 52                                               |
| Mg <sup>2+</sup>            | 71           | 50                                               |
| Ba <sup>2+</sup>            | 78           | 63                                               |

## COMPARATIVE EXAMPLE 2

Using the catalysts supported on the carriers NH<sub>4</sub>-Y and Ni-Y wherein the final nickel content of each is approximately equal, hydrogenative ring opening reaction was performed under the same conditions as those described in Example 2 to compare the catalytic performance of the respective carriers. The results are shown in Table 6.

It is apparent from Table 6 that nickel should be added to the zeolite Y through ionexchange for the best result.

Table 6

| Catalyst                 | Percent yield of monocyclic aromatics and decalin |
|--------------------------|---------------------------------------------------|
| Ni-W/NH <sub>4</sub> -Y* | 50**                                              |
| Ni-W/Ni-Y*               | 70.5**                                            |

\*The final nickel content is approximately equal

\*\*The yield was taken 10 hours after the charge stock was passed over the catalysts.

## EXAMPLE 6

Using various hydrocarbon fractions as the charge stocks, hydrogenative ring opening reaction was performed in the presence of the catalyst of the present invention and the catalyst commercially available, respectively.

The catalyst (Ni-W-V/Ni-Y) of the present invention which was prepared according to the same procedure as the catalyst preparation procedure (2) as stated above contained 2.2 weight percent sodium, 16.2 weight percent nickel, 1.6 weight percent tungsten and 1.6 weight percent vanadium.

The commercial catalyst consisted of Ni-W/SiO<sub>2</sub>.Al<sub>2</sub>O<sub>3</sub> for use in hydrogenative ring opening and contained 6.5 weight percent nickel and 20.0 weight percent tungsten, calculated as the respective metal oxides.

The treatment conditions are shown in Tables 7, 8 and 9. Further, the range of the boiling point of the charge stock was determined according to ASTM-D-86-66, and the type of the hydrocarbon was analyzed according to ASTM-D-2425-65T.

Table 7

| Run No.                                          | 1                 | 2                   | 3                 | 4                   |
|--------------------------------------------------|-------------------|---------------------|-------------------|---------------------|
| Treatment condition                              |                   |                     |                   |                     |
| Temperature (°C)                                 | 380               |                     |                   | 400                 |
| Pressure (kg/cm <sup>2</sup> )                   | 80                |                     |                   | 100                 |
| LHSV* (hr <sup>-1</sup> )                        | 2                 |                     |                   | 2                   |
| H <sub>2</sub> /charge oil (Nm <sup>3</sup> /KL) | 800               |                     |                   | 800                 |
| Catalyst                                         | Present invention | Commercial catalyst | Present invention | Commercial catalyst |
| Properties and analysis                          |                   |                     |                   |                     |
| Boiling range IBP(°C)                            | 217               | 52                  | 150               | 175                 |
| 50% (°C)                                         | 265               | 235                 | 249               | 294                 |

Table 7-continued

| Run No.                                               | 1      | 2      | 3      | 4      |
|-------------------------------------------------------|--------|--------|--------|--------|
| FBP (°C)                                              | 310    | 305    | 310    | 403    |
| Specific gravity (15/4°C)                             | 0.891  | 0.845  | 0.853  | 1.012  |
| Refractive Index ( $n_p^{20}$ )                       | 1.5062 | 1.4724 | 1.4770 | 1.5662 |
| Total sulfur (weight %)                               | 1.12   | 0.05   | 0.06   | 0.09   |
| Molecular weight                                      | 201    | 180    | 190    | 159    |
| Properties and analysis                               |        |        |        |        |
| Type of hydrocarbon<br>(mass spectrometry) (weight %) |        |        |        |        |
| Paraffin                                              | 33.6   | 51.5   | 49.0   | —      |
| Olefin                                                | 5.6    | —      | —      | —      |
| Naphthalene                                           | 10.4   | 16.1   | 21.3   | 33.8   |
| Monocyclic paraffin                                   | (6.7   | (10.5  | (13.4  | (17.9  |
| Dicyclopentane                                        | 2.8    | 4.1    | 7.0    | 13.9   |
| Tricyclic paraffin                                    | 0.9    | 1.5    | 0.9    | 2.0    |
| Monocyclic aromatics                                  | 23.4   | 27.5   | 23.4   | 38.7   |
| Alkylbenzene                                          | (12.8  | (17.0  | (12.0  | (23.2  |
| Indane, tetralin, etc.)                               | 8.8    | 10.0   | 9.9    | 11.8   |
| $C_{n}H_{2n-10}$                                      | 1.8    | 0.5    | 1.5    | 22.5   |
| Bicyclic aromatics                                    | 26.2   | 4.8    | 6.1    | 57.5   |
| Naphthalene                                           | (19.7  | (3.1   | (4.1   | (43.4  |
| $C_{n}H_{2n-14}$                                      | 4.9    | 1.4    | 1.6    | 8.0    |
| $C_{n}H_{2n-16}$                                      | 1.6    | 0.3    | 0.4    | 6.1    |
| Tricyclic aromatics                                   | 0.8    | 0.1    | 0.2    | 3.8    |
|                                                       |        |        |        | 0.4    |
|                                                       |        |        |        | 1.7    |

\*Liquid-Hourly-Space-Velocity

Table 8

| Run No.                                               | 11            | 12     | 13                   | 14     |
|-------------------------------------------------------|---------------|--------|----------------------|--------|
| Treatment condition                                   |               |        |                      |        |
| Temperature (°C)                                      |               | 400    |                      | 420    |
| Pressure (kg/cm <sup>2</sup> G)                       | Charge oil    | 100    |                      | 100    |
| LHSV (hr <sup>-1</sup> )                              | Heavy gas oil | 2      |                      | 2      |
| $H_2/\text{charge oil (Nm}^3/\text{KL)}$              | (THGO)        | 800    | Vacuum gas oil (VGO) | 800    |
| Catalyst                                              |               |        |                      |        |
| Properties and analysis                               |               |        |                      |        |
| Boiling range IBP (°C)                                | 242           | 65     | 99                   | 297    |
| 50 % (°C)                                             | 307           | 272    | 290                  | 378    |
| FBP (°C)                                              | 364           | 346    | 354                  | 445    |
| Specific gravity (15/4°C)                             | 0.852         | 0.803  | 0.814                | 0.907  |
| Refractive Index ( $n_p^{20}$ )                       | 1.4750        | 1.4540 | 1.4575               | 1.4961 |
| Total sulfur (weight %)                               | 1.22          | 0.08   | 0.06                 | 1.53   |
| Molecular weight                                      | 245           | 220    | 2323                 | 345    |
| Type of hydrocarbon<br>(mass spectrometry) (weight %) |               |        |                      |        |
| Paraffin                                              | 50.5          | 61.2   | 56.1                 | 49.2   |
| Naphthalene                                           | 23.7          | 20.8   | 28.1                 | 22.1   |
| Monocyclic paraffin                                   | (14.7         | (15.3  | (18.6                | (10.4  |
| Dicyclopentane                                        | 6.6           | 4.3    | 7.3                  | 6.9    |
| Tricyclic paraffin                                    | 2.4           | 1.2    | 2.2                  | 4.8    |
| Monocyclic aromatics                                  | 13.2          | 14.7   | 12.6                 | 9.0    |
| Alkylbenzene                                          | (7.0          | (10.2  | (6.8                 | (2.3   |
| Indane, tetralin, etc.                                | 3.8           | 4.0    | 3.8                  | 4.1    |
| $C_{n}H_{2n-10}$                                      | 2.4           | 0.5    | 2.0                  | 3.6    |
| Bicyclic aromatics                                    | 10.6          | 2.8    | 2.8                  | 14.7   |
| Naphthalene                                           | (6.0          | (1.5   | (1.5                 | (6.3   |
| $C_{n}H_{2n-14}$                                      | 3.0           | 1.0    | 0.9                  | 4.1    |
| $C_{n}H_{2n-16}$                                      | 1.6           | 0.3    | 0.4                  | 4.3    |
| Tricyclic aromatics                                   | 2.0           | 0.3    | 0.4                  | 5.0    |
|                                                       |               |        |                      | 0.9    |
|                                                       |               |        |                      | 1.2    |

Table 9

| Run No.                                  | 15               |
|------------------------------------------|------------------|
| Treatment condition                      |                  |
| Temperature (°C)                         | Charge oil       |
| Pressure (kg/cm <sup>2</sup> G)          | Asphalt cracked  |
| LHSV (hr <sup>-1</sup> )                 | distillate light |
| $H_2/\text{charge oil (Nm}^3/\text{KL)}$ | oil              |
| Catalyst                                 | —                |
| Properties and analysis                  |                  |
| Specific gravity (15/4°C)                | 1.067            |
| Refractive Index ( $n_p^{20}$ )          | 1.6318           |
| Total sulfur* (weight %)                 | 7.9              |
| Paraffin                                 | 0                |
| Monocyclic aromatics                     | 29.7             |
| Alkylbenzene                             | (20.4            |
| Indane, tetralin, etc.                   | 2.9              |
| $C_{n}H_{2n-10}$                         | 6.4              |
| Bicyclic aromatics                       | 60.5             |
|                                          | 44.4             |
|                                          | (26.2            |
|                                          | 12.3             |
|                                          | 5.9              |

Table 9-continued

| Run No.                                                                                  | 15                   |                      |
|------------------------------------------------------------------------------------------|----------------------|----------------------|
| Treatment condition                                                                      |                      |                      |
| (Naphthalene<br>(C <sub>n</sub> H <sub>2n-14</sub><br>(C <sub>n</sub> H <sub>2n-16</sub> | 33.0<br>14.9<br>12.6 | 25.7<br>11.8<br>11.4 |
| Tricyclic aromatics                                                                      | 9.8                  | 6.7                  |
| Distillation test                                                                        |                      |                      |
| 1 BP                                                                                     | 230°C                | 118°C                |
| 20 %                                                                                     | 264                  | 241                  |
| 50 %                                                                                     | 285                  | 275                  |
| 70 %                                                                                     | 306.5                | 295                  |
| EP                                                                                       | 350 (91 %)           | 354 (97.7)           |

\*According to MCTS method

### REFERENCE EXAMPLE

Several products resulting from the hydrogenative ring opening reaction of Example 6 were subjected to tubular furnace steam thermal cracking in a tube. The results of the mass balance are shown in Table 10.

Table 10

| Thermal cracking condition                                  |                           |                           |
|-------------------------------------------------------------|---------------------------|---------------------------|
| Temperature (°C)                                            | 800                       | 800                       |
| Pressure (kg/cm <sup>2</sup> G)                             | 1.0                       | 1.0                       |
| Kind of charge oil                                          | Experiment 11 product oil | Experiment 12 product oil |
| Charge oil                                                  | Mass balance<br>100.0     | 100.0                     |
| Top gas (Hydrogen)                                          | 13.3<br>(0.8)             | 13.0<br>(0.8)             |
| (Methane)                                                   | (12.5)                    | (12.2)                    |
| Ethane                                                      | 3.6                       | 3.8                       |
| Ethylene                                                    | 25.7                      | 24.9                      |
| Propylene                                                   | 13.2                      | 12.6                      |
| Others C <sub>3</sub>                                       | 0.8                       | 0.8                       |
| 1,3-butadiene                                               | 3.5                       | 3.5                       |
| Others C <sub>4</sub>                                       | 3.8                       | 3.7                       |
| Cracked gasoline (C <sub>5</sub> -C <sub>8</sub> aromatics) | 22.1<br>(12.4)            | 20.9<br>(11.8)            |
| Heavy fraction                                              | 14.0                      | 16.8                      |
| Total                                                       | 100.0                     | 100.0                     |

### What we claim is:

1. A process for conversion of a hydrocarbon fraction containing at least 10 % by weight of condensed-ring polycyclic aromatic hydrocarbons which comprises hydrogenative ring opening and hydrocracking of said polycyclic aromatic hydrocarbons by hydrogen into substantially monocyclic aromatics and saturated

cyclic hydrocarbons in the presence of a catalyst comprising 1 to 25% of nickel, 1 to 20% of tungsten and 0.1 to 5% of vanadium, based on the total weight of a carrier plus the three metals supported on said carrier, which carrier consists of an NaY zeolite in which more than 60 molar % of sodium ions have been exchanged with nickel ions.

2. A process according to claim 1 wherein said catalyst comprises 6 to 20% of nickel, 1 to 10% of tungsten and 1 to 2% of vanadium, based on the total weight of the carrier plus the three metals.

3. The process according to claim 1 wherein the catalyst is sulfided prior to the hydrogenative ring opening reaction.

4. The process according to claim 3 wherein the sulfiding is effected by heating the catalyst in an atmosphere comprising hydrogen and vapor of a sulfide.

5. The process according to claim 1 wherein the exchange of sodium ions of the zeolite Y is effected by exchanging the sodium ions with ammonium ions in an aqueous solution and then exchanging the ammonium ions with nickel ions in an aqueous solution.

6. The process according to claim 5 wherein the ammonium ions are provided by a water soluble ammonium salt which yields ammonium ions in an aqueous solution.

7. The process according to claim 6 wherein the ammonium salt is ammonium chloride.

8. The process according to claim 5 wherein the nickel ions are provided by a water-soluble nickel salt which yields nickel ions in an aqueous solution.

9. The process according to claim 8 wherein the nickel salt is selected from the group of nickel chloride and nickel nitrate.

\* \* \* \* \*